

L. LORENTOWICZ.  
COMPOSITION FOR REPAIRING SCORED CYLINDERS.  
APPLICATION FILED JUNE 13, 1916.

1,239,195.

Patented Sept. 4, 1917.



Fig. 1.

Fig. 3.



Fig. 2.

Fig. 4.



Fig. 5.



Inventor

Leonard Lorentowicz.

Witness

Poland T. Booth

By

F. Dittmar

Attorney

# UNITED STATES PATENT OFFICE.

LEONARD LORENTOWICZ, OF IRVINGTON, NEW JERSEY.

## COMPOSITION FOR REPAIRING SCORED CYLINDERS.

1,239,195.

Specification of Letters Patent.

Patented Sept. 4, 1917.

Application filed June 12, 1916. Serial No. 103,453.

*To all whom it may concern:*

Be it known that I, LEONARD LORENTOWICZ, a citizen of the United States, residing at Irvington, county of Essex, State of New Jersey, United States, have invented certain new and useful Improvements in Compositions for Repairing Scored Cylinders, of which the following is a specification, reference being had therein to the accompanying drawing.

The invention relates to improvements in compositions for renewing and repairing worn metal surfaces, and more particularly for filling of scores and the like occurring in engine cylinders, principally the cylinders of internal combustion engines.

It is well known that a great many cylinders of internal combustion engines are damaged by wear and very often they are scored to a considerable extent by foreign matter getting into the cylinder, or by parts of the apparatus becoming disarranged and scratching or gouging the interior of the cylinder wall so that there is no tight fit between the piston and the cylinder, and this of course prevents maximum compression, and the engine soon becomes useless, or its efficiency very greatly impaired. This scoring is very often done by reason of a wrist pin coming loose and being carried along by the piston in a manner to scrape the interior wall of the cylinder, so that it becomes channeled or scored.

It has heretofore been the practice to repair scored cylinders by grinding or reboring them, and this is a very slow method and is expensive because of the time required for the purpose, and such manner of repairing necessitates the use of a new size piston and ring. Another method has been to weld the scored parts to the cylinder, but in subjecting the cylinder to a welding heat, the same becomes warped, and therefore, in the majority of instances, requires grinding or reboring, and a second disturbing of the contour of the inside of the cylinder wall.

The main object of the invention is to provide a composition for the purpose, and one which, while being easily and readily applied to, or incorporated in, the part of the surface to be repaired, is of a nature to withstand the maximum temperatures to which it may be subjected, and which are common to engine cylinders in their operation.

With these and other objects in view, the

invention resides in the certain new and useful composition to be hereinafter more fully described, set forth in the appended claims, and the manner of its application illustrated in the accompanying drawings, in which:

Figure 1 is a fragmentary top view of a conventional form of cylinder showing scores occurring in the inner surface of the same, ready for the filling,

Fig. 2 is an enlarged fragmentary section of the inner wall showing the surface thereof, when repaired,

Fig. 3 is a second enlarged fragmentary section of the inner wall showing natural scores prior to the preparation of the same for filling, and

Fig. 4 is a similar view showing the scores prepared, filled, and completed, and

Fig. 5 is a similar view showing another form of natural score occurring in the wall of the cylinder.

In producing the composition of the present invention, I use block-tin alone, or in combination with either or both of the following metals, namely, silver, copper, depending upon the type of engine cylinder, or other metal surface, it is desired to repair, some of such surfaces being subjected to greater temperatures than are others, as in the case of air or water-cooled cylinders, the surface of the cylinder is heated to a lesser degree than is a cylinder not provided with a cooling medium, so that the several ingredients may be varied to produce a composition filling of a desired or predetermined melting point. However, it has been determined that the block-tin may be used alone, in some instances, and its melting point is to be increased or decreased, as may be desired, by adding thereto either or both of the other metals mentioned, and, preferably in a proportion of one-half per cent., or from one half to one per cent. of the latter metals.

However, while preferring to make up the composition, in the proportions above stated, it is to be understood that I do not specifically limit myself thereto, as slight variations will not seriously interfere with the efficiency of the composition, and are to be considered within the scope of the present invention.

To illustrate the application of the desired composition, reference being had to the drawings in which is shown the conventional form of cylinder A with an inner wall B,

and an outer wall C forming between them, a water space D through which water is circulated to keep the cylinder cool under running conditions, this water being supplied by the usual water circulating system with which all water cooled engines are equipped and which is understood by those skilled in the art, and for that reason is not explained in detail here. The face E, of the inner wall 10 B, is in contact with the piston or packing rings of the piston which operate within the cylinder, and it frequently happens that this wall E becomes scored in different ways, and very often by the ends of a wrist pin which comes loose and such scoring is shown at F in Fig. 1. This scoring is sometimes quite extensive, and such extensive scoring is shown in Figs. 1 and 2. If the old method 15 of welding is resorted to, the cylinder is subjected to a high heat which very often warps it, and the cylinder then requires reborning, and I have devised means and method for filling the scored parts without the application of a high heat, such as is necessary in 20 the welding process.

After thoroughly cleaning the surface of a score in the metal surface, by scraping the same lightly to remove the top grease and dirt therefrom, and until the same brightens 30 to a shiny finish, a suitable flux is applied, and then the score is filled with the composition, in either molten or solid state, and is then thoroughly amalgamated, or otherwise incorporated in position, and is finished 35 flush with the contour of the surface, by means of a suitable tool, scraper or special machine (not shown). In the application of the composition, a suitably heated soldering iron, or a small torch is used to furnish 40 just sufficient heat to keep the same in thoroughly melted or workable state, without any undue heating of the surrounding surface, and, in some instances, it is desired that the surfaces of a score be prepared with 45 a thin coating of tin, to insure the adherence of a relatively hard alloy or composition thereto.

In any case, the invention provides for a metallic composition having a high melting point so that it is not affected, after it is placed in the cylinder, by the degree of heat generated by the combustion of the fuel in the engine cylinder. I have found that a very good metal for this purpose is

block-tin, and this is to be further hardened, 55 when desired, by the addition of from one-half to one per cent. of either or both of the other metals hereinbefore mentioned.

The drawing in Fig. 2 shows the scored parts F filled with the metal G. The metal 60 is put into the grooves, and is then scraped, with a scraper or similar tool, or special machine devised for the purpose, (not shown), shaped to the contour of the cylinder wall so that it is substantially concentric and 65 flush with the surface E of the cylinder. It is usual to first apply to the cleaned surface of a score a suitable flux so that the metal attaches itself well to the metal of the cylinder, such flux consisting of acid and sal-ammoniac, or any other of the usual fluxes 70 that are used in soldering operations.

In Fig. 3 I have shown the cylinder wall B provided on its face E with grooves H, which are shown small in proportion to the 75 thickness of the wall of the cylinder, being virtually small scratches. When these scratches occur and it is desired to fill them with metal, I deepen the scratches, that is, I score them to a greater extent so 80 that a larger area is presented for the fastening of the metal G, which metal is shown in Fig. 4, after it is applied to the scratches H, which have been deepened, as shown at I in said Fig. 4. I have found that this metal, 85 when applied and reduced to the contour of the wall of the cylinder, forms a smooth surface, and cylinders so treated have given long service without any leaking between the piston and the cylinder. The metal is 90 of a high melting point so that the running of the engine does not furnish enough heat to cause the filling to melt, and this is particularly true, in the case of a water cooled 95 engine.

Having thus fully described the invention, what I claim, is:—

A composition for repairing scored metallic surfaces adapted to be subjected to relatively high temperatures, which consists 100 of block tin, silver and copper, substantially in the proportions described.

In testimony whereof I affix my signature in the presence of two witnesses.

LEONARD LORENTOWICZ.

Witnesses:

RICHARD E. SMITH, Jr.,

ROBERT GRUBER.